

May 19, 1931.

W. J. MOELLER ET AL

1,805,739

BUILT-UP ROOFING AND METHOD OF APPLICATION

Filed March 29, 1926



Wm. J. Moeller Inventor  
Arthur N. Zimmerman Inventor  
By their Attorney  
Teal & Mills, Jr.

## UNITED STATES PATENT OFFICE

WILLIAM J. MOELLER, OF MOUNT HEALTHY, AND ARTHUR H. ZIMMERMAN, OF LOCKLAND, OHIO, ASSIGNORS TO THE PHILIP CAREY MANUFACTURING COMPANY, A CORPORATION OF OHIO.

## BUILT-UP ROOFING AND METHOD OF APPLICATION

Application filed March 29, 1926. Serial No. 98,327.

Our invention relates to built-up roofing and method of application thereof. Heretofore built-up roofing has been applied by the application on the roof of a sheet or layer of 5 bituminous saturated paper or felt and then mopping over such layer a hot bituminous bonding and protective material applying a second layer, mopping over that a second application of hot bituminous bonding and 10 protective material and continuing the application of the saturated felt or paper and the hot bituminous bonding and protective material until the desired thickness of roofing has been applied. Such method and application of roofing requires facilities for heating the bituminous material which is usually done on the ground and then the hot material is raised in pails or buckets to 15 the roof where it was mopped on or applied by the workman. This method has many objections including the cost of heating and handling the bituminous material. It is difficult by this method to get the coating of the hot bituminous material evenly applied 20 over the surface and to prevent air pockets or bubbles being formed, due to air being entrapped, in the hot bituminous material. While it is being mopped on the roofing preparatory to the application of the next above 25 sheet of saturated paper or felt. We have overcome the objections to this method of application, and, have provided a built-up roofing which is superior to and more easily applied than the built-up roofings heretofore 30 known in the art, have dispensed with the use of heating facilities, thereby reducing the cost of application and obtaining a more uniform built-up roofing, having provided a more even distribution of the bituminous 35 material between the layers, and have overcome the objectionable entrapment of air bubbles or air pockets between layers of the saturated felt or paper. By our invention 40 we provide a sheet or paper saturated or impregnated with bituminous material such as heretofore used for built-up roofings and form on one or both sides and integral therewith a coating of a bituminous material such as asphalt, coal tar, etc., which is distributed evenly over the sheet of saturated 45 50 55 60 65 70 75 80 85 90 95 100

felt or paper in the factory. The coating which we prefer to use is a bituminous material of a character that when cool or at atmospheric temperature will permit the sheet of saturated paper or felt upon which the coating is applied to be rolled without cracking and which will not crack when the paper is unrolled. Such coating is to be of a character that a liquid solvent applied to its surface by a mop, a brush, or a light spray, will dissolve the surface of the coating so as to provide a tacky or adhesive surface to which the next sheet or ply of saturated paper or felt will adhere. We also provide for use with the roofing material referred to a solvent which can be readily applied either by brush, mop, or spray to the surface of the coating. Such solvent is preferably one with a high solvent power so that a very small quantity will readily cause the surface of the coating to become tacky or adhesive. Such solvents as naptha, gasoline and kerosene have been found satisfactory for bituminous coatings of asphalt. We however do not limit ourselves to the use of asphalt as a saturant or coating or the use of the solvents referred to as any suitable coating can be used and any solvent suitable for the purpose of dissolving the coating may be used. Among other solvents for asphalt which could be used are benzol, tol-nol, wood turpentine, wood creosote oil, carbon tetrachloride.

In the drawing we have shown a cross section of a built up roof in which A, A, A, are layers of bituminous saturated felt or like roofing material. B is a coating on the top of the felt of bituminous material such as asphalt. C is a similar coating on the bottom of the saturated felt A, which coating C is of like material to the coating B. The coating layers B and C are applied to the saturated felt A in the factory and the roofing material is rolled and forwarded to the place of application. By our method of application the solvent is applied to either or both of the coatings B and C as the roll of roofing material is being laid. This solvent would be applied as shown in the drawing to the right of the roll of material.

which forms the top ply of roofing. As the solvent is applied to either or both of the coatings B and C and the material is brought into contact by unrolling of the roofing material, the coatings which are in a tacky or adhesive condition securely hold the layers of saturated material together. By our method of application we have a built-up roof composed of the desired number of plies of saturated roofing material bonded together by a distinct layer of bituminous material.

Our method of application of built-up roofings is as follows: The roofing materials having been prepared in the factory by saturating and coating a sheet of satisfactory material the first ply, layer or sheet of saturated and coated roofing material is laid and fixed in place by nailing or if it is desired may be cemented to the roof, in which case we preferably use a saturated roofing material which has been coated on both sides and as the roll is laid over the roof a solvent is applied by the workman to the surface of the coating on the under side of the sheet thereby partially dissolving same and causing its surface to become adhesive and tacky. The result is that when the tacky or adhesive surface comes in contact with the roof it cements itself thereto and becomes fixed in place. The next above layer of saturated and coated roofing material is then applied by having the workman mop the cold solvent on the surface of the first layer just ahead of the roll of the second layer of saturated and coated roofing material as it is being unrolled so that the coating on the upper surface of the first sheet is partially dissolved, and the surface becomes tacky or adhesive and readily cements itself to the second layer as it is unrolled and brought into contact with the coating on the first layer. In this way it will be seen that the roll of roofing material as it is unrolled passes over the portion of the material that is being cemented to the next below layer and thereby tends to force out any bubbles, and prevent the formation of air pockets between the layers. The third layer of felt is applied in a similar manner and likewise the fourth, and fifth depending on the number required. The coating having been applied in the factory will be of even thickness and the result will be a more uniform thickness of the finished built-up roofing. If it is desired to form on the surface of the roof a gravel or granular surface such result may be obtained in two ways, either the coating on the upper surface may be dissolved by the solvent being applied so as to make the coating tacky or adhesive and then the gravel or granular material applied, or if desired the top ply could be a layer of granular surfaced roofing material having the granular material applied thereby more

evenly distributing the granular material. If desired a roller could be passed over each layer as it was applied to supply the additional weight to roll the layer, being applied, on to the layer to which it was being applied.

Claim—

The method of forming upon a roofing support a built up roofing of layers of bituminous saturated sheets alternated with layers of a bituminous substance which comprises coating both sides of a saturated sheet with a layer of bituminous material of the desired thickness, forming the coated sheet, after the coating is set, into a roll, unrolling the roll onto the roofing support while applying a solvent to the coated sheet material slightly in advance of the line of tangency between the roll and the roofing support, then unrolling a second roll of the coated sheet material while applying a solvent to the surface of the material slightly in advance of the line of tangency between the roll and the upper surface of the first sheet, whereby in applying the sheet material to the surface below, any air bubbles or surplus solvent will be forced out from between the approaching surfaces due to the curvature of the sheet being applied and the weight of the unrolled portion of the sheet.

In testimony whereof, we have signed our names to this specification.

WILLIAM J. MOELLER.  
ARTHUR H. ZIMMERMAN.

100

105

110

115

120

125

130